

# UNITED STATES PATENT OFFICE.

FREDERICK C. OVERBURY, OF HILLSDALE, NEW JERSEY, ASSIGNOR, BY MESNE ASSIGNMENTS, TO THE FLINTKOTE COMPANY, OF BOSTON, MASSACHUSETTS, A CORPORATION OF MASSACHUSETTS.

## MINERAL-SURFACED ROOFING MATERIAL.

1,238,805.

Specification of Letters Patent.

Patented Sept. 4, 1917.

No Drawing.

Application filed January 20, 1917. Serial No. 143,502.

*To all whom it may concern:*

Be it known that I, FREDERICK C. OVERBURY, a citizen of the United States, residing at Hillsdale, in the county of Bergen and 5 State of New Jersey, have invented new and useful Improvements in Mineral-Surfaced Roofing Material, of which the following is a specification.

This invention relates to roofing fabrics 10 of the type in which the exposed facing or coating consists of a relatively thick layer of crushed slate or analogous mineral material partially embedded in a layer of pitch, asphalt, or equivalent waterproof compound. 15 In such fabrics, the foundation consists of a sheet of felt or other fibrous material saturated or impregnated with a bituminous or hydrocarbon compound, and on this compound so treated is applied a layer of pitch 20 or asphalt or the like, in which the crushed mineral is embedded while said layer is in a plastic adhesive condition. Such roofings, in the form of sheets, strips or shingles, are 25 in great demand because of their rough appearance and due to the color effects produced by the mineral facings.

In manufacturing and marketing such goods, I have found that it frequently happens that the appearance of the fabric is 30 injured due to the fact that certain oily or greasy components of the saturating or coating compounds reach the mineral material and discolor it in spots or patches. Further, when different batches of the fabric or 35 roofing are held in stock, even though formed of the raw material, they differ in tint or shade, and, when laid on the same roof, produce unsatisfactory results.

In an earlier application, Serial No. 40 56,289, filed October 16, 1915, I pointed out a method of curing the trouble. As a result of further investigations and experimentation, I have discovered that, in lieu of spraying or otherwise treating the mineral 45 surface with the specific materials referred to in said application for preventing the oily components of the bituminous or hydrocarbon saturating or coating components from discoloring the rough mineral

surface, I am able to secure still better results by employing dextrin as the main component of the surface-treating material. I preferably mix dextrin with hot water in the proportion of 1.6 pounds of dextrin to enough water to produce one gallon of the 55 mixture, although these proportions may be changed as desired. In case there should be any tendency for the dextrin to grow sour or to spoil, any suitable preservative, such as bichlorid of mercury, may be used. If 60 used, I do not employ the described preservative in large amounts, as one part thereof to two thousand parts of the dextrin solution is sufficient.

As soon as the mineral-surfaced roofing 65 fabric is produced, I treat it with the dextrin solution, either by spray, or with a brush, or by dipping the surface in the solution, or applying the solution thereto by a roll. The solution spreads over the sheet in 70 a thin film which does not mask the rough mineral surface, or act as a binder, but prevents the oily components from creeping over the slate or mineral particles and discoloring them. The film of the dextrin, 75 when the water has evaporated, is transparent, and it also acts to prevent the sticking of one sheet of the fabric to the other when the sheets are superimposed. Of course any equivalent for dextrin may be 80 used in its stead without departing from the scope of this invention.

Having thus explained the nature of my invention and one way of producing the desired results, without setting forth all of the 85 embodiments of the invention and the different ways in which it may be practised, what I claim is:

1. A weatherproof roofing fabric, having a bituminous coating and a layer of crushed 90 mineral partially embedded therein, and having a film of dextrin on said crushed mineral.

2. The herein-described process which consists in treating the crushed-mineral face of 95 a mineral-surfaced roofing fabric with a liquid containing dextrin, to leave a film of dextrin thereon.

3. The herein-described process which consists in treating the crushed-mineral face of a mineral-surfaced roofing fabric with an aqueous solution of dextrin to leave a film of dextrin thereon.

4. The herein-described process which consists in treating the crushed-mineral face of

a mineral-surfaced roofing fabric with an aqueous solution of dextrin, and a preservative for the dextrin to leave a film of dextrin <sup>15</sup> thereon.

In testimony whereof I have affixed my signature.

FREDERICK C. OVERBURY.